

(No Model.)

J. A. COLEMAN.  
HORSESHOE NAIL.

No. 397,896.

Patented Feb. 19, 1889.



FIG. 1.



FIG. 5.



FIG. 9.



FIG. 2.



FIG. 3.



FIG. 4.



FIG. 10.



FIG. 6.



FIG. 7.



FIG. 8.

WITNESSES.

*John H. Hogan,  
William H. Barron*

INVENTOR.

*John A. Coleman*

# UNITED STATES PATENT OFFICE.

JOHN A. COLEMAN, OF PROVIDENCE, RHODE ISLAND.

## HORSESHOE-NAIL.

SPECIFICATION forming part of Letters Patent No. 397,896, dated February 19, 1889.

Application filed April 21, 1887. Renewed July 25, 1888. Serial No. 281,022. (No model.)

*To all whom it may concern:*

Be it known that I, JOHN A. COLEMAN, a citizen of the United States, residing at Providence, in the county of Providence and State 5 of Rhode Island, have made a new and useful Invention in Horseshoe-Nails, of which the following is a specification.

My invention relates to horseshoe-nails; and it consists in the formation of a horseshoe-10 nail in a new and useful manner, substantially as hereinafter described and claimed.

In the drawings, Figure 1 is a side view of a completed horseshoe-nail produced according-15 to my invention. Fig. 2 is a cross-section of Fig. 1, through the central part of the nail, on the dotted line  $x'x$  of Fig. 1. Fig. 3 is a cross-section through the portion of the nail where the head and body parts join, on the dotted line  $y'y$  of Fig. 1; and Fig. 4, a cross-20 section on dotted line  $y'y'$ . Fig. 5 is a side elevation, partly in section, of the punch and die apparatus for striking up the head of the nail-blank from the drawn wire used in the formation of the nail. Figs. 6 and 7 are side 25 and edge views of the headed blanks. Fig. 8 is a view of the rollers that are used for drawing down the shank and forming the point of the nail upon the blank. Fig. 9 is a side view of a piece of the drawn wire which is used to 30 form the nail-blank. Fig. 10 is a cross-section of Fig. 9 upon the dotted line  $x'x'$ .

My invention consists in using drawn wire for the manufacture of horseshoe-nails and the production of the completed horseshoe-35 nail from such drawn wire by a method which shall preserve intact the shell of hardened metal which is produced in the process of drawing wire upon its exterior, and surrounds a central core of softer and ductile metal within 40 the body of the wire. In Figs. 2, 3, and 10 I have represented this exterior shell surround-45 ing the internal core of the wire as somewhat thickened or exaggerated in proportion and terminating more abruptly at its lines of junction with the core than it actually is in the wire, for the better illustration of the same. I first take the piece of wire cut off of suitable length to form the blank shown in Figs. 6 and 7, and place it in the dies shown in 50 Fig. 5, and strike up the head of the horse- shoe-nail upon it, thus forming a blank. This striking up is done by an endwise com-

pression of the metal. This process causes the outer shell, as well as the ductile core 55  $b$  of the drawn wire, to be entered into and united with the head of the nail, so as to become homogeneous with it, and so as to impart the strengthening and stiffening properties of the outer shell to the point of junction between the head and shank of the 60 nail, where the strain of the shoe comes upon it when it is driven into the hoof through the shoe in the usual manner. It also leaves the shank of the blank with its hardened outer shell portion and internal ductile core so 65 nearly the size of the finished nail that the subsequent drawing-down processes required to give the shank its ultimate form in the finished nail are so slight as not to impair or injure the outer hardened shell which the drawn 70 wire had in the outset. I next take the nail-blank so formed by the heading-up process, and, placing it between the rollers shown in Fig. 8, I draw down the shank and point of the nail thereby. In accomplishing this drawing- 75 down process I finish off the point of the nail by cold-rolling, with sufficient pressure to give it the requisite hardness and stiffness throughout its entire structure; but I apply only sufficient pressure to the shank part of the nail 80 above the point in rolling it down to reduce it to the proper form without destroying the softness and ductility of the core of the wire employed.

Any clipping or cutting of the point of the 85 nail to reduce it to proper form should be confined entirely to the point portion, which is hardened throughout by the rolling process, and not be extended into the hardened shell surrounding the ductile core above the point. 90 By thus drawing the nail down from the blank I leave the soft and ductile core of the latter surrounded by the original tubular hardened shell of the wire the entire length of the nail from within its head to its hardened-point 95 portion, thereby producing a shank of the nail having superior stiffness for driving into the hoof to secure the shoe upon it without impairing the capacity of the ductile central core to endure clinching over the hoof in the usual manner after the nail has been driven in. All parts of the shank of the nail being 100 surrounded by this hardened outer shell of the wire, which is incorporated into and ho-

mogeneous with the head of the nail at one end and with the hardened point of the nail at the other end, and is unbroken and unimpaired from the head to the point on all sides 5 of the core, it is impossible for the nail to split in driving into the hoof.

I am aware that horseshoe-nails have heretofore been cut from a nail-plate which was previously cold-rolled upon the opposite surfaces 10 and that these cold-rolled opposite surfaces formed in the finished nail so cut from the plate hardened shells or walls upon two sides of the plate, between which was a soft and ductile core, thus stiffening the nail-shank 15 to some extent; but the opposite hardened surfaces in this nail were separated at the edges of the nail where it was cut from the plate by the soft central core lying between them, and they differed from my nail in having no outer hardened-shell portion along the 20 edge uniting the shell portion upon the opposite surfaces of the nail, and were consequently not so stiff and more liable to bend in driving into the hoof, as well as to allow the hardened shell portions upon the opposite faces to 25 split off from the nail.

I am also aware that horseshoe-nails have been produced by taking a soft-iron blank cut from hot-rolled metal and rolling down the shank part and point of the nail therefrom by 30 more or less cold-rolling, which produces a partially-hardened shell around the central ductile core; but the shell so produced differs from that upon my nail in not having the same 35 thickness where the head and shank part of

the nail unite, and in not being incorporated in the intimate manner with the head part which exists in the nail formed by me, as hereinbefore described.

My nail also differs from nails in which the shanks are reduced by hammering or compression while hot, in the superior stiffness of the shank, due to the outer hardened inclosing-shell thereof, which does not exist in nails thus formed. 40

Instead of using drawn wire rectangular in cross-section, other forms of drawn wire may be employed and reduced to the form required in the finished nail by suitable compression upon it at different points, which 45 will leave the outer shell of the wire surrounding the ductile core portion of the nail intact and incorporated with the head and point portion thereof, substantially as hereinbefore described. 50

What I claim as new and of my invention is—

As a new article of manufacture, a horseshoe-nail formed of drawn wire by the process of striking up and enlarging the head of 60 the nail therefrom and drawing down the shank and hardened-point portion therefrom without substantially impairing the hardened shell of the wire which surrounds the ductile central core portion of the nail, substantially 65 as described.

JOHN A. COLEMAN.

Witnesses:

JOHN W. HOGAN,  
WILLIAM H. BARRON.